

## UNITED STATES PATENT OFFICE

HENRY C. GARDINER, OF ANACONDA, MONTANA

## GRANULATED PRODUCT AND PROCESS FOR MAKING SAME

No Drawing.

Application filed August 22, 1927. Serial No. 214,791.

This invention relates to a granulated product and a process for making the same.

An object of the invention is the provision of a process for granulating or increasing 5 the size of finely divided particles which make up such arsenical materials as flue dust, bag house dust, chamber dust, dust produced from the well known Cottrell installation, hot and cold treater dust and all similar materials or 10 products which result from the metallurgical reduction of arsenic bearing ores and materials.

Another object of the invention is the provision of a process for producing aggregates 15 of fine particles resulting from the metallurgical reduction of arsenic bearing ores so that the product may be handled more expeditiously and with the elimination of dust.

A further object of the invention is the 20 provision of a process for granulating fine particles of dust resulting from the metallurgical reduction of arsenic bearing ores while at the same time controlling the solubility of the granules thus formed.

25 A still further object of the invention is the provision of a process for granulating fine particles of dust resulting from the metallurgical reduction of arsenic bearing ores while increasing the weight per unit volume 30 of the dust thus simplifying and reducing the cost of packing.

This invention will be best understood from a consideration of the following detailed description; nevertheless it is to be understood 35 that the invention is not confined to the disclosure, being susceptible of such changes and modifications which shall define no material departure from the salient features of the invention as expressed in the appended 40 claims.

In carrying out my invention I mix sulphuric acid and water with one or more of the following products,—finely divided particles of flue dust, bag house dust, chamber 45 dust, dust produced from the well known Cottrell installation, hot and cold treater dust, and all similar materials or products which result from the metallurgical reduction of arsenic bearing ores and materials. The mixing 50 is accomplished easily and economically

in an apparatus such as a pug mill or a granulator. Any type of mill suitable for the purpose may be employed. The dusts are first tested in order to determine the percentage of arsenical products. Depending upon the 55 purpose for which the product is adapted to be used, a dust may be mixed with a different kind of dust mentioned above for the purpose of increasing the percentage of the arsenical products or for decreasing the percentage. 60

The quantity of the sulphuric acid used is governed by the degree of firmness, relative solubility of the toxic components and the quantity of free sulphuric acid desired in 65 the finished product. From one to twenty percent by weight of sulphuric acid may be added. These percentage limits will give a sufficiently wide range of degrees of firmness, free sulphuric acid and solubility of the toxic 70 components in the product that such product may be very efficaciously utilized in the preservation of wood or articles formed of wood which are ordinarily buried or partially buried in the ground and which are subject to the 75 attacks of fungi, bacteria and insects.

The quantity of water added is dependent upon the type of equipment employed for the purpose of granulation. Ordinarily it is only necessary to add sufficient water to produce 80 a granulated product in which the granules are of the desired size whereby they will not adhere either to each other or to the granulating and drying equipment. It has been found that as low as five percent of water 85 by weight will be sufficient to accomplish the desired result. The percentage limits of water are approximately from five to twenty per cent.

The mixing of the sulphuric acid and water 90 in the proper percentages with one or a mixture of two or more of the products resulting from the metallurgical reduction of arsenic bearing ores and materials may be easily accomplished in a manner that the process will 95 be continuous. The sulphuric acid may be added first and then the water may be supplied in the proper proportion or vice versa. If desired the sulphuric acid and water may be carefully mixed and this mixture may be 100

added directly to the arsenic containing material either in the pug mill or granulator or before the materials have been placed in the apparatus.

5 The mixing of the sulphuric acid and water with one or a mixture of two or more of the arsenic containing products is done for the particular purpose of providing wet granules of the desired size. The mixture 10 is then dried in any type of apparatus suitable for the purpose. A drier of the type commonly known as a rotary dryer or rotary kiln has been found to be most suitable for such a purpose, since the rotary motion produces granules of very firm texture.

15 While I have stated that sulphuric acid and water are employed within certain ranges of percentages it will be appreciated that other solutions, simple, colloidal or denatured, may be employed for the purpose.

20 Solutions containing starch or sugar, or glues, and flour may be used for the purpose. One such sugar containing substance found to work very effectively is refuse or 25 stock molasses.

25 After the dust has been thoroughly mixed with the sulphuric acid water it is then dried in any suitable manner, as by means of the usual drying equipment.

30 I claim:—

1. A process for granulating dust resulting from the metallurgical reduction of arsenic bearing ores and material which comprises mixing said dust with sulphuric acid 35 and water, agitating and at the same time drying the mixture.

2. A process for granulating dust resulting from the metallurgical reduction of arsenic bearing ores and material which comprises mixing said dust with sulphuric acid 40 and then water, agitating and at the same time drying the mixture.

3. A process for granulating dust resulting from the metallurgical reduction of arsenic bearing ores and material which comprises mixing said dust with from one to 45 twenty percent by weight of sulphuric acid and from five to twenty percent by weight of water, agitating and at the same time drying the mixture.

4. A process for granulating dust resulting from the metallurgical reduction of arsenic bearing ores and material which comprises mixing said dust with from one to 55 twenty percent of sulphuric acid and sufficient water to cause granulation of the dust, agitating and at the same time drying the mixture.

5. A product of the class described comprising a granulated dust formed from a mixture of a dust resulting from the metallurgical reduction of arsenic bearing ores, sulphuric acid and water.

6. A product of the class described comprising a granulated dust formed from a

dried mixture of a dust resulting from the metallurgical reduction of arsenic bearing ores, sulphuric acid and water.

7. A product of the class described comprising pellets formed of a mixture of an aqueous solution of sulphuric acid and a dust resulting from the metallurgical reduction of arsenic bearing ores.

8. A product of the class described comprising pellets formed of a mixture of arsenic bearing materials, sulphuric acid and water, said acid acting as a binder for the arsenic bearing material.

9. A product of the class described comprising pellets formed of arsenic bearing materials and sulphuric acid, the acid acting as a binder for the arsenic bearing material.

10. A process of manufacturing a wood preservative which comprises mixing dust resulting from the metallurgical reduction of arsenic bearing ores and materials with sulphuric acid and water, and drying the mixture with agitation to form granules while varying the solubility in water of the toxic components of the dust.

HENRY C. GARDINER.

95

100

105

110

115

120

125

130